

Aug. 23, 1949.

R. O. DENYES  
TREATMENT OF VISCOSE CELLULOSE  
FILAMENTARY MATERIALS  
Filed Nov. 29, 1945

2,479,605



## UNITED STATES PATENT OFFICE

2,479,605

TREATMENT OF VISCOSE CELLULOSE  
FILAMENTARY MATERIALSRussell Owens Denyes, Rome, Ga., assignor, by  
mesne assignments, to Celanese Corporation of  
America, a corporation of Delaware

Application November 29, 1945, Serial No. 631,729

3 Claims. (Cl. 8—137.5)

1

This invention relates to the purification of freshly formed regenerated cellulose products, especially of those which have been regenerated from viscose, and has for its object the provision of certain improvements in the initial stages of the purification treatment. The freshly formed viscose products contain adherent and occluded acid picked up from the regenerating bath, together with appreciable amounts of reaction products, comprising carbon disulfide, elemental sulfur, salts and metallic sulfides. These require removal in a process generally known as purification. A particularly detrimental impurity is lead sulfide, derived from the lead linings of the coagulating bath conduits. Purification generally comprises a sequence of treatments, such as washing with warm water to remove the adherent and occluded acid and water soluble salts, and to distill out the occluded carbon disulfide, treating with a sulfur solvent, such as an aqueous solution of sodium sulfide or of ammonium sulfide, and finally rinsing with lukewarm water. Washing with plain water and desulfurizing with alkaline sulfide solutions do not effectuate complete removal of the metallic sulfides. Since these tend to discolor the viscose products, it is the practice of the art to subject the products subsequently to a bleaching treatment as, for example, with chlorine water or with sodium hypochlorite solutions. Such bleaching treatments, however, result in partial degradation of the viscose product due to the unavoidable oxidizing action on the regenerated cellulose of the bleaching agent employed.

This invention is concerned with the initial washing step in the purification procedure, and has for its object the provision of an improved method of washing freshly formed viscose products, for example, freshly spun filaments, whereby the normal impurities with the exception of elemental sulfur, are effectually removed. The conventional subsequent bleaching treatment is rendered unnecessary, and no increase in process time is involved. In accordance with the invention, viscose filaments may be purified while in the gel state in the form of bobbin spinning packages, pot spun cakes, staple fiber tow, or while passing over the initial thread-storage, thread-advancing devices of continuous spinning machines.

I have found that viscose filaments in the gel state, while still wet with adherent acid carried off from the spinning bath, may be purified to a high degree of whiteness without bleaching in the conventional sense, without implicating a

2

significant extension of existing purification schedules and without significant impairment of the tensile characteristics, if the water which is normally employed for washing out the acid is dosed with relatively small amounts of certain chemicals, namely, alkali-metal chlorites, chlorine dioxide or chlorous acid, used singly or preferably, conjointly with a sequestering agent, such as sodium hexametaphosphate.

10 For convenience, the invention will be described with reference to the purification of viscose yarn while on the bobbin on which it was spun. It is, of course, understood that the invention is applicable to the purification of viscose filaments 15 in the gel state when produced under other types of spinning. In accordance with the method of the invention, the purification may be carried out by employing a series of separate washes and using a solution containing sodium chlorite at the start of the initial wash of the yarn, for example, during the preliminary acid-removal wash. If the yarn is highly discolored, I may obtain a more satisfactory color removal in a short period of time by the use of a sequestering 25 agent, such as sodium hexametaphosphate, in conjunction with the sodium chlorite. It is sometimes advantageous to employ a short initial acid-removal wash prior to the addition of sodium chlorite when purifying a yarn package that 30 washes slowly. In this way the bulk of the acid is removed from the yarn prior to its exposure to the chlorite ions, and this minimizes the danger of over-exposure and slight damage to the yarn resulting therefrom. When employing an initial 35 wash, the time must be adjusted so that the acidity of the spin package does not drop below the required level prior to completion of the action of the chlorite. This is important since the acidity required for the most effective action 40 of sodium chlorite, in this type of operation, is furnished by the acid remaining in the yarn from the spinning operation.

While the acid may be washed out in the initial wash to any desired extent, it is desirable in 45 certain instances to effect a more certain control over the acidity of the filaments and the treating solution by employing an initial wash of such duration that most of the acid is removed from the spin package. The yarn is then further washed with a precisely acidified solution of sodium chlorite. The initial wash and the second wash may or may not contain a sequestering agent, such as sodium hexametaphosphate, depending upon the nature and degree of the dis- 50 coloration of the yarn and the extent of bleach-

ing required. Very effective results in the way of color removal may be accomplished by using a small amount, say 0.1%, of sodium hexametaphosphate in the initial acid-removal wash. Such a wash is preferably carried out at a temperature around 60° C. A hot solution is most effective when using sodium chlorite alone or in conjunction with sodium hexametaphosphate in the initial wash.

The optimum duration and the temperature of the initial wash and of the second wash, concentration of the chlorite or chlorine dioxide, concentration of the sequestering agent, if employed, in either or both the initial wash and second wash, and acidity of the yarn or second wash are all dependent upon the degree of discoloration of the yarn, the extent of purification required, and the form of the yarn at the time of treatment, i. e., type of yarn package. It is generally desirable to use a temperature in excess of 40° C., preferably between 50° C. and 60° C. Excellent results on a highly discolored yarn have been obtained using concentrations of sodium chlorite between 0.5 and 1.0 g. per liter. Specific cases may require somewhat higher concentrations, or permit the use of lower concentrations of this compound. Concentrations of 0.5 to 1.0 g. per liter of sodium hexametaphosphate have proven definitely advantageous in some cases. When an acidified purification solution is employed, the preferred acidity of said solution is at least pH 5.5 or more strongly acid.

Sodium chlorite in an acid solution attacks certain metals, even stainless steel, and the resulting corrosion products may impair the color of the yarn. It is advisable to protect the metal from these agents and I have found that bobbins and the like coated with a Bakelite lacquer, such as Heresite, are suitably protected.

In order to make accurate comparisons between viscose filaments treated according to the invention, untreated viscose filaments and bleached viscose filaments, evaluation measurements were made by means of a General Electric recording spectrophotometer. The results of the invention will, accordingly, be better understood with reference to the accompanying drawing which is a composite reproduction of the recordings of the spectrophotometer.

The following examples illustrate applications of this invention to purifying viscose yarn on a spin bobbin:

#### EXAMPLE I

A very satisfactory color removal and uniform whiteness was obtained as follows using 150/40 bright viscose yarn:

Purification schedule minutes  
 0.1% sodium hexametaphosphate (57° C.) 100  
 0.1% sodium hexametaphosphate 0.065% sodium chlorite 0.005% sulfuric acid (57° C.) 150  
 Hot water (57° C.) 200  
 Ammonium sulfide (40° C.) 100  
 Hot water (57° C.) 100

The yarn package may be characterized as follows:

Weight of yarn (dry basis) pound 1  
 Thickness of yarn cake mm 19  
 Length of package—outside mm 130  
 Length of package—inside mm 180  
 Rate of flow gal/min 0.01

#### EXAMPLE II

Same as Example I except that the sodium hexametaphosphate was omitted from the initial

hot water wash (100 min.) which preceded the chlorite treatment.

#### EXAMPLE III

Bobbin purification schedules in minutes on 150/40 bright viscose yarn

| Conventional Process | Treatment of Invention |
|----------------------|------------------------|
| 50 HW                | 100 HW                 |
| 200 HW               | 150 SS                 |
| 100 HW               | 200 HW                 |
| 100 A                | 100 A                  |
| 20 HW                | 20 HW                  |
| 80 HW                | 80 HW                  |

HW = hot (50° C.) water.

SS = hot (50° C.) sodium chlorite (0.07%), sodium hexametaphosphate (0.1%), sulfuric acid to give pH 4.5-5.5 after addition of sodium chlorite.

A = ammonium sulfide (0.35%) at 45° C.

20 A package produced from the same viscose and spun under identical conditions as in the "Conventional Process" yarn was drip-bleached with chlorine water in accordance with the treatment of United States Patent 2,064,300 and used for 25 whiteness comparison.

Both the yarns of Example III, the drip-bleached yarn, and a well bleached commercial yarn were cone wound, sampled and a test fabric of each was prepared by knitting 24" swatches.

30 These fabrics were tested on a General Electric recording spectrophotometer for whiteness in comparison with magnesium oxide. For purposes of comparison similar tests were made to show the relative whiteness with reference to a high

35 grade of chemically refined wood pulp. By chemically purified wood pulp is meant the so-called high-alpha dissolving pulp such as is used as a source of cellulose in preparation of viscose. The readings of the spectrophotometer are

40 shown in the composite graphs of the accompanying drawing. It is significant to note that the whitest yarns now produced are less white than the cellulose pulp from which the yarn is produced. This indicates the extent of discoloration 45 caused by the viscose process.

I claim:

1. The method of purifying freshly formed viscose cellulose filamentary materials, which comprises subjecting the materials, while in a gel state and while still containing adherent acid from the coagulating bath, to washing treatments with an aqueous solution containing sodium hexametaphosphate and then with an aqueous solution of sodium hexametaphosphate and a compound selected from the group consisting of alkali-metal chlorites, chlorine dioxide and chlorous acid, the acidity of the latter aqueous solution being at least pH 5.5.

2. The method of purifying freshly formed viscose cellulose filamentary materials, which comprises subjecting the materials, while in a gel state and while still containing adherent acid from the coagulating bath, to washing treatments with an aqueous solution containing sodium hexametaphosphate and then with an aqueous solution of sodium hexametaphosphate and sodium chlorite, the acidity of the latter aqueous solution being at least pH 5.5.

3. The method of purifying freshly formed viscose cellulose filamentary materials, which comprises subjecting the materials, while in a gel state and while still containing adherent acid from the coagulating bath, to washing treatments at a temperature of 40 to 60° C. with an aqueous solution of sodium hexametaphosphate and then

with an aqueous solution containing sodium chlorite and sodium hexametaphosphate, the sodium chlorite and sodium hexametaphosphate being each present in said latter aqueous solution in a concentration of from 0.5 to 1.0 grams per liter, the acidity of the latter aqueous solution being at least pH 5.5, and then subjecting the products to desulfurizing and washing treatments.

RUSSELL OWENS DENYES

REFERENCES CITED

The following references are of record in the file of this patent:

UNITED STATES PATENTS

| Number    | Name   | Date          |
|-----------|--------|---------------|
| 1,633,220 | Mendel | June 21, 1927 |
| 1,646,625 | Mendel | Oct. 25, 1927 |

| Name     | Date          |
|----------|---------------|
| Thurmond | Oct. 16, 1934 |
| Fiske    | Feb. 25, 1936 |
| Hall     | Dec. 13, 1938 |
| Fryer    | Dec. 2, 1941  |
| Jackson  | Apr. 17, 1945 |

FOREIGN PATENTS

| Country       | Date          |
|---------------|---------------|
| Switzerland   | Aug. 16, 1937 |
| Great Britain | 1935          |

OTHER REFERENCES

Munter et al., Application of Sodium Metaphosphate to Textile Processes, Am. Dyes. Rep. Jan. 28, 1935, pages 40-47. (Copy in 8-82.)  
 Matthews, Bleaching and Related Processes, 1921, Chem. Cat. Co., N. Y., pages 471-473. (Copy in Div. 43.)